

# UNITED STATES PATENT OFFICE.

WALTER C. SMITH, OF ROSELLE, NEW JERSEY, ASSIGNOR TO UNITED STATES SMELTING, REFINING & MINING COMPANY, A CORPORATION OF MAINE.

## METHOD OF MAKING COPPER-CADMIUM ALLOY.

1,307,642.

Specification of Letters Patent. Patented June 24, 1919.

No Drawing.

Application filed August 15, 1918. Serial No. 249,924.

To all whom it may concern:  
Be it known that I, WALTER C. SMITH, a citizen of the United States, residing at Roselle, in the county of Union and State 5 of New Jersey, have invented certain new and useful Improvements in Methods of Making Copper-Cadmium Alloy; and I do hereby declare the following to be a full, clear, and exact description of the invention, 10 such as will enable others skilled in the art to which it appertains to make and use the same.

The invention relates to the production of copper cadmium alloys.

15 It has been found that the addition of a small amount of cadmium (say from  $\frac{1}{2}$  to 1.1 per cent.) to copper which does not injuriously affect its ductility approximately doubles its tensile strength at ordinary temperatures, while reducing its conductivity but approximately 5 to 15 per cent. A copper cadmium alloy having a small percentage of cadmium is therefore well adapted for the manufacture of wire for use as 20 electric conductors, particularly under conditions where the available supports may be widely separated. The usual methods of producing copper alloys are however wholly unsuited to the production of copper cadmium 25 alloy containing an approximately definite percentage of cadmium, owing to the characteristics of cadmium which cause its rapid volatilization and oxidation when added to a molten copper bath with such 30 resulting rapid and variable losses of cadmium as to preclude the production of even an approximately uniform alloy. It is the primary object of the present invention in its entirety to provide for the commercial 35 production of a copper cadmium alloy containing a comparatively low percentage of cadmium. The complete method by which such production is rendered feasible includes a two stages, each of which constitutes a 40 feature of the invention, and by each of which a copper cadmium alloy of substantially uniform and known composition may be produced.

The method or sub-method comprising the 45 first stage is used to produce an alloy the melting point of which is below the boiling point of cadmium, and consequently containing a higher percentage of cadmium than

should be present in an alloy to be used in the manufacture of electric wires, since the 55 melting points of alloys containing less than 5 per cent. of cadmium are above the boiling point of cadmium. A small quantity of an alloy having a known high percentage of cadmium (say from thirty to seventy-five 60 per cent. or more) such as may be produced by the first stage is utilized in the method or sub-method of the second stage to produce an alloy having a low percentage of cadmium and therefore well adapted for the uses 65 above indicated.

To produce the high-percentage cadmium alloy with comparatively little and approximately unvarying loss of cadmium, the temperature and the melting point of a molten 70 bath of copper are simultaneously and quickly reduced to a point below the boiling point of cadmium by adding solid cadmium to the bath, either as a metal or as a high-percentage cadmium alloy. The heat absorbed in melting the cadmium (or alloy) 75 rapidly reduces the temperature of the bath, while the melting point of the alloy produced by the mixture of the cadmium and the copper rapidly falls as the proportion of 80 the cadmium increases. The addition of between five and seven per cent. in weight of cadmium to the copper bath should reduce its temperature and its melting point to a 85 temperature below the boiling point of cadmium, (about 700° C.) During the addition of this amount of cadmium there will of course be more or less loss, due to its volatilization during the interval in which the temperature of the bath remains above 90 the boiling point of the cadmium. The cadmium should therefore be added as rapidly as is practicable, and in proper condition as to size and distribution of pieces or lumps to avoid freezing the bath. The supply of 95 heat to the bath should also be shut off before adding the cadmium to secure the best results. Thus far the method will give a copper cadmium alloy having between 5 and 10 per cent. of cadmium. If an alloy having a higher percentage of cadmium is desired, as will be the case if the alloy is to 100 be used in making a low percentage alloy in accordance with the second stage of the invention, the additional cadmium required 105 is added to the bath while maintaining the

temperature of the bath between its melting point and the boiling point of cadmium. As soon as the cadmium is melted and thoroughly mixed with the copper, the bath is cast into solid form.

While the cadmium may be added either as a metal or as an alloy, it is better practice to add to the copper bath a sufficient amount of previously made alloy having a high percentage of cadmium, to bring the temperature of the bath below the boiling point of cadmium, since this will result in less violent disturbance in the bath and less loss of cadmium. After the temperature of the bath has been thus reduced below the boiling point of cadmium, the percentage of cadmium in the bath may best be brought up to the point desired by adding cadmium metal. The temperature of the bath, even after it has been reduced below the boiling point of cadmium, is still above that at which cadmium will burn (about 350° C.), and consequently there may be some loss of cadmium, due to oxidation and burning during the addition of the cadmium and the stirring of the bath to thoroughly mix the alloy or the cadmium with the copper. This loss may be reduced or prevented by protecting the bath with a molten cover of neutral material, such as a flux, by powdered charcoal, or other suitable cover, which will prevent oxidation and burning of the cadmium at the surface of the bath.

To produce an alloy having a comparatively low percentage of cadmium, and consequently a melting point above the boiling point of cadmium, a comparatively small quantity of copper cadmium alloy having a comparatively high percentage of cadmium is added to a molten bath of copper, the resulting alloy being cast as soon as possible after the melting and mixing of the added alloy. The percentage of cadmium in the added alloys should be so high that the quantity requisite to secure the desired percentage of cadmium in the bath will be a small proportion of the bath, since to avoid loss of cadmium the added alloys should be melted in the least possible time by the absorption of heat from the bath. Satisfactory results have been obtained by the use of alloys having from 30 to 75 per cent. of cadmium. Loss of cadmium, due to oxidation and burning at the surface of the bath, may be prevented or reduced, as in the first stage of the method, by providing the bath with a molten protective covering of neutral material, or with a protective covering of powdered charcoal.

In utilization of the method for the production of a copper cadmium alloy for use in the manufacture of electric-conductor wire, it will probably be found undesirable to produce an alloy having more than 1.1 per

cent. cadmium, since an increase in the percentage of cadmium beyond this point so reduces the ductility as to render rolling and drawing of the alloy difficult, if not impracticable. An alloy containing from .8 to 1.1 per cent. cadmium has given the most satisfactory results. In producing alloy for electric wires care should be taken that no zinc nor tin are present in the copper bath, since the presence of these metals, even in small quantities, materially lowers the conductivity of the alloy. If the low percentage cadmium alloy is not to be used for the manufacture of electric conductors, the presence of more than 1.1 per cent. of cadmium or the presence of small quantities of zinc or tin, or possibly other metals, in the alloy produced may not be undesirable.

What is claimed is:—

1. The method of making copper cadmium alloy which consists in simultaneously reducing the temperature and the melting point of a molten copper bath to a temperature below the boiling point of cadmium by the addition thereto of cadmium in a solid state, thereafter continuing the addition of cadmium while maintaining the bath at a temperature above its melting point and below the boiling point of cadmium, solidifying the resulting alloy, and thereafter adding to a molten bath of copper a quantity of the solidified alloy which is a small proportion of the total bath.

2. The method of making copper cadmium alloy which consists in simultaneously reducing the temperature and the melting point of a molten copper bath to a temperature below the boiling point of cadmium by the addition thereto of cadmium in a solid state, thereafter continuing the addition of cadmium while maintaining the bath at a temperature above its melting point and below the boiling point of cadmium until the bath contains a comparatively high percentage of cadmium (say thirty to seventy-five per cent. or more), solidifying the resulting alloy, and thereafter adding to a molten copper bath a quantity of the high percentage alloy sufficiently small to be melted by heat absorbed from the bath and thereby produce an alloy having a comparatively low percentage of cadmium, (say one or two per cent.).

3. The method of making copper cadmium alloy which consists in simultaneously reducing the temperature and the melting point of a molten copper bath to a temperature below the boiling point of cadmium by the addition thereto of cadmium in a solid state.

4. The method of making copper cadmium alloy which consists in simultaneously reducing the temperature and the melting point of a molten copper bath to a temperature below the boiling point of cadmium by

the addition thereto of cadmium in a solid state, and thereafter continuing the addition of cadmium while maintaining the bath at a temperature above its melting point and below the boiling point of cadmium.

5. The method of making copper cadmium alloy which consists in simultaneously reducing the temperature and the melting point of a molten copper bath to a temperature below the boiling point of cadmium by the addition thereto of a solid alloy having a high percentage of cadmium.

10 6. The method of making copper cadmium alloy which consists in simultaneously reducing the temperature and the melting point of a molten copper bath to a temperature below the boiling point of cadmium by the addition thereto of a solid alloy having a high percentage of cadmium, and thereafter continuing the addition of cadmium to the bath while maintaining the bath at a temperature above its melting point and below the boiling point of cadmium.

15 7. The method of making copper cadmium alloy which consists in providing a molten bath of copper with a neutral cover, and simultaneously reducing the temperature and the melting point of the bath to a tem-

perature below the boiling point of cadmium by the addition thereto of cadmium in a solid state.

8. The method of making copper cadmium alloy which consists in adding to a molten bath of copper, cadmium in a solid state sufficiently small in quantity to be melted by heat absorbed from the bath and sufficiently high in cadmium to reduce the temperature of the bath to a point below the boiling point of cadmium and above the melting point of the resulting bath.

10 9. The method of making copper cadmium alloy which consists in adding to a molten bath of copper solid cadmium alloy having a high percentage of cadmium in such small quantity that the added alloy may be melted by heat absorbed from the bath.

20 10. The method of making copper cadmium alloy which consists in providing a molten bath of copper with a neutral cover and adding to the bath solid copper cadmium alloy having a high percentage of cadmium in such small quantity that the added alloy may be melted by heat absorbed from the bath.

WALTER C. SMITH.